

# UNITED STATES PATENT OFFICE.

WILLIAM H. OCKLESTON, OF BOURN, AND THOMAS BURNELL CARMICHAEL, OF WATERLOO, NEAR LIVERPOOL, ENGLAND.

## TANNING.

1,413,488.

Specification of Letters Patent. Patented Apr. 18, 1922.

No Drawing.

Application filed January 21, 1922. Serial No. 530,955.

To all whom it may concern:

Be it known that we, WILLIAM HENRY OCKLESTON and THOMAS BURNELL CARMICHAEL, subjects of the King of Great Britain, residing, respectively, in Bourn, in the county of Cambridge, England, and Waterloo, near Liverpool, in the county of Lancaster, England, have invented certain new and useful Improvements Relating to 10 Tanning, of which the following is a specification.

This invention relates to improvements in tanning and has reference to a process for fixing vegetable and mineral tannages with 15 the object of shortening the period of drying, more particularly in the case of vegetable tanned leather, and this without darkening or streaking the surface.

According to the invention the hides or 20 the like after being subjected to the tannage are treated with an aqueous solution of pyridine which fixes the tanning agent and permits washing and subsequent rapid drying without liability for the tanning agent to 25 bleed or sweat out and so cause a darkening or streaking of the surface.

When a vegetable tanning agent is used the washing is effected in a weak acid solution.

30 The strength of the pyridine solution would be varied in accordance to the kind of hides to be treated and the quality desired in the resulting product, and in average cases would be about 10 to 25 per cent.

35 Hides after being subjected in the usual manner to, say, vegetable tanning agents, and before oiling are treated with the pyridine solution in which they are soaked for, say, four to twelve hours; the hides may

40 then be washed without loss of the tanning substances; as stated, when a vegetable tanning agent is employed the washing is carried out with a weak acid condition, say a 5% solution. A 5% aqueous solution of

45 oxalic acid forms an excellent washing solution, but weak solutions of other organic acids, such as formic acid, may be employed for washing, and in some cases inorganic acids, say sulphuric acid may be used for

50 acidifying the washing solution.

After treatment with the pyridine the tanning agent in the hides or the like is not soluble in the washing solution, so that there is no loss of the tanning agent in the wash- 55 ing. The use of the acid washing solution also has the effect of brightening the colour

of the resulting leather. The hides are oiled in the usual manner after washing.

After washing, the hides are rapidly dried in, say, a hot stove, the product being uniform in colour and there being little risk of the darkening or streaking which results in the ordinary processes, in consequence of the tanning material coming to the surface, especially when the attempt is made to shorten the period of drying.

In the case, for example, of alum tannage, the hides after the alum treatment are transferred to the pyridine solution for a suitable period, usually from four to twelve hours; 70 this treatment fixes the alum so that the hides may be washed without loss of alum and without the resulting hardening of the leather such as occurs in the ordinary process of alum tannage.

We also find that though the chrome in chrome tanning is not so liable to be washed out as is the case with other tannages, a better fixing and resulting product is obtained by the pyridine treatment.

Having now particularly described and ascertained the nature of our said invention, and in what manner the same is to be performed, we declare that what we claim is:

1. A method of tanning which includes 85 the step of subjecting the material being tanned to the action of pyridine.

2. A method of tanning which includes the step of subjecting the material being tanned to the action of an aqueous solution 90 of pyridine and washing with acid solution.

3. A method of tanning which includes the step of subjecting the material being tanned to the action of a ten per cent solution of pyridine.

4. A method of tanning which includes the step of subjecting the material being tanned to the action of pyridine, and then treating the material with oxalic acid.

5. A method of tanning which includes 100 the step of subjecting the material being tanned to the action of pyridine and then treating the material with 5 per cent oxalic acid.

In testimony whereof we affix our signatures in presence of two witnesses.

W. H. OCKLESTON.  
THOMAS BURNELL CARMICHAEL.

Witnesses:

JOSEPH E. HIRST,  
MARGUERITA JONES.